# EUROPEAN PATENT SPECIFICATION

(11) **EP 3 269 840 B1**
(45) Date of publication and mention of the grant of the patent: **14.04.2021**
(21) Application number: 17180675.5
(22) Date of filing: 11.07.2017
(51) Int. Cl.: C23C 10/20, C23C 10/60

(54) **METHOD OF CHROMIZING AN ARTICLE INCLUDING INTERNAL PASSAGES OF THE ARTICLE**
VERFAHREN ZUR CHROMIERUNG EINES ARTIKELS, EINSCHLIESSLICH DER INNENDURCHFÜHRUNGEN DES KÖRPERS
PROCÉDÉ DE CHROMISATION D'UN OBJET, Y COMPRIS SES PASSAGES INTERNES

(30) Priority: 12.07.2016 US 201615207745
(43) Date of publication of application: 17.01.2018
(73) Proprietor: Raytheon Technologies Corporation, Farmington, CT 06032 (US)
(72) Inventor: TASK, Michael N., Vernon, CT 06066 (US)
(74) Representative: Dehns

(56) References cited:
- EP-A2- 1 548 156
- WO-A1-2015/108766
- US-A- 5 128 179
- US-A1- 2010 151 125

## Description

### BACKGROUND

Articles that are subject to corrosion, such as gas turbine engine components, may include a coating to protect an underlying material from corrosion. Some articles have internal passages which are subject to corrosion and can be protected by such a coating.

Various techniques can be used to deposit a coating, such as "chromizing," which results in a chromium-rich coating. Chromizing can be accomplished by, for instance, a vapor deposition process, or by the application of a slurry containing active chromium to the article and processing it.

WO 2015/108766 A1 discloses methods of applying chromium diffusion coatings onto selective regions of a component.

US 2010/151125 A1 discloses a slurry chromizing process.

### SUMMARY

From a first aspect, the invention provides a method for chromizing an article as recited in claim 1.

In an embodiment, the slurry flows into the internal passages.

In a further embodiment of any of the foregoing embodiments, the amount of solids in the slurry is greater than about 25 percent by weight of the slurry.

In a further embodiment of any of the foregoing embodiments, the amount of solids in the slurry is between about 50 and about 75 percent by weight of the slurry.

In a further embodiment of any of the foregoing embodiments, the residue-removal agent is inert with respect to the article and the slurry (in the heating).

In a further embodiment of any of the foregoing embodiments, the residue-removal agent forms a matrix during the heating. The matrix traps the residue.

In a further embodiment of any of the foregoing embodiments, the slurry contains an amount of residue-removal agent sufficient to form a continuous matrix of residue-removal agent during the heating step.

In a further embodiment of any of the foregoing embodiments, the slurry contains an amount of solids, and greater than about 50% by weight of the solids of the residue removal agent.

In a further embodiment of any of the foregoing embodiments, the article is an airfoil.

In a further embodiment of any of the foregoing embodiments, the article is cleaned with a hot pressurized cleaning solution in a pressure chamber.

### BRIEF DESCRIPTION OF THE DRAWINGS

The various features and advantages of the present disclosure will become apparent to those skilled in the art from the following detailed description. The drawings that accompany the detailed description can be briefly described as follows.
Figure 1A illustrates an example article.
Figure 1B illustrates schematically illustrates a section view of the example article with internal passages.
Figure 2 illustrates a method of chromizing the example article.
Figure 3 illustrates the example article with chromizing residue and a chromium-enriched coating.
Figure 4A illustrates the cleaned example article with a chromium-enriched coating.
Figure 4B illustrates a section view of the cleaned example article with a chromium-enriched coating.
Figure 5 illustrates a schematic detail view of a matrix formed by residue removal agent on the example article.

### DETAILED DESCRIPTION

Figure 1A illustrates an example article 10. In this example, the article 10 is an airfoil for a gas turbine engine. The article 10 may potentially be exposed to hot corrosion during the operation of the gas turbine engine, for example, up to temperatures of about 1900° F (1038° C). The article 10 may be formed of steel or a superalloy, such as a cobalt- or nickel-based superalloy. It should be understood, however, that this disclosure will benefit other articles or gas turbine engine components with internal passages. Figure 1B illustrates a representative section view of the article 10 with internal passages 12.

Figure 2 illustrates a method 100 of chromizing the article 10 including the internal passages 12. In Step 102, a slurry is applied at least to the internal passages 12. The slurry can be applied by, for example, dipping the article 10 into the slurry, spraying the slurry onto the article 10, painting the slurry onto the article 10, flowing the slurry across the article 10 and into internal passages 12, or by another method of application. Although some of the slurry may drip off, the slurry at least forms a slurry coating on surfaces of the internal passages 12.

The slurry contains an active coating metal of chromium powder in liquid carrier material. The slurry may also include alumina powder and/or a diffusion activator, such as chromium (III) chloride or a halide activator. The amount of liquid carrier material controls the viscosity of the slurry. The slurry contains enough liquid carrier material such that the slurry can readily flow through internal passages 12 of article 10. In one example, the amount of solids in the slurry is between about 50 and 75 percent by weight of the slurry. The slurry also includes residue-removal agent, silica, which is discussed in more detail below.

In Step 104, the article 10 with slurry coating is heated to diffuse chromium from the slurry coating into the article 10 as represented at D (Figure 3, discussed in more detail below). In one example, the heating is conducted in a furnace having a continual flow of argon to produce an argon environment, in which argon is the most abundant gas, at a temperature greater than 1900° F (1038°C), such as 1950° F (1066° C) to 2000° F (1094° C). The article 10 is heated for a selected amount of time, depending upon a desired thickness of the resulting chromium diffusion coating. In some examples, the selected amount of time is between 6 and 16 hours and the final chromium diffusion coating includes at least 20% by weight of chromium. The heating and diffusion creates a chromium-enriched coating 16, but leaves a residue or crust 14 on a surface 15 of the article 10 or internal passages 12, as shown in Figure 3. For example, the coating 16 is the surface region of the article 10 that has diffused chromium.

In Step 106, the article 10 is processed to remove the residue 14 from the article 10, yielding an article 10 with the chromium-enriched coating 16 having a clean surface 16a, as is shown in Figures 4A-4B. For example, as will be discussed in more detail below, the processing includes cleaning the article with a cleaning solution. The coating 16 can be on an outer surface of the article 16 and/or on the surfaces 15 of the internal passages 12, as shown in Figures 4A-B, respectively. In this example, the residue 14 is removed from the article 10 with a hot, pressurized cleaning solution. The cleaning solution is a hydroxide, and, in one example, the processing step is performed inside a pressure chamber, such as an autoclave.

The residue removal agent permits removal of the residue 14. The residue removal agent is thermodynamically inert with respect to the slurry and the article 10. That is, the residue removal agent does not react or substantially react with the slurry or the article 10. The residual removal agent is silica (silicon dioxide).

Turning to Figure 5, the residue-removal agent 18 forms a matrix 20 on the surface 15 of the internal passage 12 during the heating step 104. Though the surface of the internal passage 12 is shown in Figure 5, it should be understood that the residue removal agent 18 can form a matrix 20 on the exterior surface of the article 10 as well. For instance, the heating diffuses the chromium into the article 10 and evaporates the liquid carrier, leaving the silica to consolidate on the surface 15. The consolidated silica forms the matrix 20 and traps the residue 14. For example, the residue 14 may be residual constituents of the powders in the slurry, byproducts of the powders, or foreign substances.

The residue removal agent 18 is soluble in the cleaning solution. In one example, the residue 14 is insoluble or substantially insoluble in the cleaning solution. When the residue-removal agent 18 is dissolved by the cleaning solution, it releases the residue 14 from the article 10. This cleaning solution can flow through the internal passages 12 to contact the residue 14 in the internal passages 12 and thereby remove the residue 14. Other residue-removal methods, such as grit blasting or a similar mechanical process, can be difficult to perform in internal passages 12 or other non-line-of-sight surfaces of an article 10 because such methods require a clear physical line-of-sight to a surface for effective removal.

In one example, the slurry contains an amount of residue removal agent 18 sufficient to form the matrix 20. In a further example, the slurry contains an amount of residue removal agent 18 sufficient to form a continuous matrix 20. That is, the continuous matrix 20 entraps all the residue 14 from the heating and diffusion, and when the matrix 20 is removed from the article 10 by the processing step 106, substantially all of the residue 14 is removed with it. Although less residue removal agent 18 could be used, lower amounts increase the potential for residue 14 to bond to the surface 15 of the internal passage 12 or to the article 10, thereby making removal more difficult. In yet another example, the slurry contains greater than about 25% by weight of solids of residue removal agent 18. More particularly, the slurry contains greater than about 50% by weight of solids of residue removal agent 18.

Although a combination of features is shown in the illustrated examples, not all of them need to be combined to realize the benefits of various embodiments of this disclosure. In other words, a system designed according to an embodiment of this disclosure will not necessarily include all of the features shown in any one of the Figures or all of the portions schematically shown in the Figures. Moreover, selected features of one example embodiment may be combined with selected features of other example embodiments.

The scope of legal protection given to this disclosure is determined the following claims.

## Claims

1. A method for chromizing an article (10), the method comprising:
applying a slurry to an article (10), the slurry including active chromium and a residue-removal agent (18), wherein the article (10) includes internal passages (12), and a residue (14) is in the internal passages (12);
heating the article (10) and slurry to diffuse chromium from the slurry into the article (10), the heating leaving the residue (14) on the article (10) with the residue-removal agent (18); and
removing the residue-removal agent (18), to thus remove the residue (14) from the article (10), using a cleaning solution, wherein the residue-removal agent (18) is soluble in the cleaning solution, wherein the residue removal agent (18) is silica and the cleaning solution is a hydroxide.

2. The method of claim 1, wherein the slurry flows into the internal passages (12).

3. The method of any preceding claim, wherein the amount of solids in the slurry is greater than 25 percent by weight of the slurry.

4. The method of any preceding claim, wherein the amount of solids in the slurry is between 50 and 75 percent by weight of the slurry.

5. The method of any preceding claim, wherein the residue-removal agent (18) is inert with respect to the article (10) and the slurry during the heating step.

6. The method of any preceding claim, wherein the residue-removal agent (18) forms a matrix (20) during the heating step, the matrix (20) trapping the residue.

7. The method of claim 6, wherein the slurry contains an amount of residue-removal agent (18) sufficient to form a continuous matrix (20) of residue-removal agent (18) during the heating step.

8. The method of any preceding claim, wherein the slurry contains an amount of solids, and greater than about 50% by weight of the solids of the residue removal agent (18).

9. The method of any preceding claim, wherein the article (10) is an airfoil (10).

10. The method of claim 1, wherein the cleaning solution is a hot pressurized cleaning solution and the article (10) is cleaned with the hot pressurized cleaning solution in a pressure chamber.

## Patentansprüche

1. Verfahren zum Chromieren eines Artikels (10), wobei das Verfahren Folgendes umfasst:
Auftragen einer Aufschlämmung auf einen Artikel (10), wobei die Aufschlämmung aktives Chrom und einen Rückstandsentferner (18) beinhaltet, wobei der Artikel (10) Innendurchführungen (12) beinhaltet und sich in den Innendurchführungen (12) ein Rückstand (14) befindet;
Erhitzen des Artikels (10) und der Aufschlämmung, um Chrom aus der Aufschlämmung in den Artikel (10) zu diffundieren, wobei das Erhitzen den Rückstand (14) mit dem Rückstandsentferner (18) auf dem Artikel (10) hinterlässt; und
Entfernen des Rückstandsentferners (18) mithilfe einer Reinigungslösung, um den Rückstand (14) so von dem Artikel (10) zu entfernen, wobei der Rückstandsentferner (18) in der Reinigungslösung löslich ist, wobei der Rückstandsentferner (18) Silica und die Reinigungslösung ein Hydroxid ist.

2. Verfahren nach Anspruch 1, wobei die Aufschlämmung in die Innendurchführungen (12) strömt.

3. Verfahren nach einem der vorstehenden Ansprüche, wobei die Menge an Feststoffen in der Aufschlämmung mehr als 25 Gewichtsprozent der Aufschlämmung beträgt.

4. Verfahren nach einem der vorstehenden Ansprüche, wobei die Menge an Feststoffen in der Aufschlämmung zwischen 50 und 75 Gewichtsprozent der Aufschlämmung beträgt.

5. Verfahren nach einem der vorstehenden Ansprüche, wobei der Rückstandsentferner (18) bezogen auf den Artikel (10) und die Aufschlämmung während des Erhitzens inert ist.

6. Verfahren nach einem der vorstehenden Ansprüche, wobei der Rückstandsentferner (18) während des Erhitzens eine Matrix (20) bildet, wobei die Matrix (20) den Rückstand einschließt.

7. Verfahren nach Anspruch 6, wobei die Aufschlämmung eine Menge eines Rückstandsentferners (18) enthält, welche ausreichend ist, um während des Erhitzens eine durchgehende Matrix (20) aus Rückstandsentferner (18) zu bilden.

8. Verfahren nach einem der vorstehenden Ansprüche, wobei die Aufschlämmung eine Menge von Feststoffen und mehr als 50 Gew. -% der Feststoffe des Rückstandsentferners (18) enthält.

9. Verfahren nach einem der vorstehenden Ansprüche, wobei der Artikel (10) ein Schaufelprofil (10) ist.

10. Verfahren nach Anspruch 1, wobei die Reinigungslösung eine heiße, unter Druck stehende Reinigungslösung ist und wobei der Artikel (10) mit der heißen, unter Druck stehenden Reinigungslösung in einer Druckkammer gereinigt wird.

## Revendications

1. Procédé de chromisation d'un objet (10), le procédé comprenant :
l'application d'une suspension sur un objet (10), la suspension comportant du chrome actif et un agent d'élimination de résidu (18), dans lequel l'objet (10) comporte des passages internes (12), et un résidu (14) se trouve dans les passages internes (12) ;
le chauffage de l'objet (10) et de la suspension pour diffuser le chrome de la suspension dans l'objet (10), le chauffage laissant le résidu (14) sur l'objet (10) avec l'agent d'élimination de résidu (18) ; et
le retrait de l'agent d'élimination de résidu (18), pour éliminer ainsi le résidu (14) de l'objet (10), à l'aide d'une solution de nettoyage, dans lequel l'agent d'élimination de résidu (18) est soluble dans la solution de nettoyage, dans lequel l'agent d'élimination de résidu (18) est de la silice et la solution de nettoyage est un hydroxyde.

2. Procédé selon la revendication 1, dans lequel la suspension s'écoule dans les passages internes (12).

3. Procédé selon une quelconque revendication précédente, dans lequel la quantité de solides dans la suspension est supérieure à 25 pour cent en poids de la suspension.

4. Procédé selon une quelconque revendication précédente, dans lequel la quantité de solides dans la suspension est comprise entre 50 et 75 pour cent en poids de la suspension.

5. Procédé selon une quelconque revendication précédente, dans lequel l'agent d'élimination de résidu (18) est inerte par rapport à l'objet (10) et la suspension pendant l'étape de

6. Procédé selon une quelconque revendication précédente, dans lequel l'agent d'élimination de résidu (18) forme une matrice (20) pendant l'étape de chauffage, la matrice (20) piégeant le résidu.

7. Procédé selon la revendication 6, dans lequel la suspension contient une quantité d'agent d'élimination de résidu (18) suffisante pour former une matrice continue (20) d'agent d'élimination de résidu (18) pendant l'étape de chauffage.

8. Procédé selon une quelconque revendication précédente, dans lequel la suspension contient une quantité de solides, et supérieure à environ 50 % en poids des solides de l'agent d'élimination de résidu (18).

9. Procédé selon une quelconque revendication précédente, dans lequel l'objet (10) est un profil aérodynamique (10).

10. Procédé selon la revendication 1, dans lequel la solution de nettoyage est une solution de nettoyage pressurisée chaude et l'objet (10) est nettoyé avec la solution de nettoyage pressurisée chaude dans une chambre de pression.
